

June 21, 1949.

W. G. ABBOTT, JR

2,473,499

PRODUCTION OF SLIVERS OF ARTIFICIAL FIBERS

Filed April 30, 1946



Inventor  
William G. Abbott Jr.  
by Robert Bushman & Crown  
att'ys.

## UNITED STATES PATENT OFFICE

2,473,499

## PRODUCTION OF SLIVERS OF ARTIFICIAL FIBERS

William G. Abbott, Jr., Milford, N. H.

Application April 30, 1946, Serial No. 666,172

6 Claims. (Cl. 18—54)

1

This invention relates to the formation of slivers of artificial fibers, and has for its principal object to provide an improved process for continuously forming a sliver of artificial fibers in which staple lengths of the fibers are overlapped and staggered longitudinally of the sliver.

My application Serial No. 506,664, filed October 18, 1943, patented as No. 2,399,191, dated April 30, 1946, describes the feeding to the plurality of orifices of an extrusion nozzle a composite of filament-forming material and another, non-filament-forming, material, with those materials so disposed that bodies of each are presented to the individual orifices at frequent intervals, the bodies of non-filament-forming material filling the orifice cross-section and thereby temporarily excluding the filament-forming material from passage through the orifice. By separating the non-filament-forming material from the filament-forming material after extrusion of the sliver, the resulting sliver comprises overlapped and longitudinally staggered staple length filaments adapted for the spinning processes with little if any further rearrangement of the staple filaments.

The present invention aims to improve upon the process of said application, Serial No. 506,664, by avoiding the necessity for inclusion of a non-filament-forming material as an element of the composite which is extruded, and also aims to improve over the process of said application by providing a more expeditious way of producing a sliver in which filaments of a plurality of different compositions are blended together.

The improved method of this application preferably comprises the preparation of a composite including one filament-forming material in a continuous phase and another filament-forming material in a dispersed phase, both of these materials being in a flowable condition and being immiscible with each other so that each retains its separate identity. In practice this condition is best secured by adjusting the relative fluidity of the filament-forming materials before putting them together, so that one of these materials is sufficiently less fluid than the other material so as to exist in the form of particles dispersed through the said other material. Stability of the dispersion is further promoted by use of dispersed particles having a different surface tension from that of the continuous material.

The drawing is a diagrammatic view showing a dispersion of bodies of one filament-forming material in another filament-forming material pass-

2

ing through an extrusion nozzle into a hardening bath, producing a sliver of staple lengths of each of the two kinds of filament-forming material, the diameters of these staple lengths being greatly exaggerated in order to permit the two kinds of fibers to be distinguished in the drawing.

The relative proportions of the filament-forming material may be adjusted within a wide range, and the proportion of one to the other will govern the proportion of one kind of filament to the other kind of filament in the extruded sliver.

A wide variety of combinations of filament-forming materials may be employed. For instance, one filament-forming material may be a protein such as the product made from casein, which is extruded to make the fiber known commercially as "Aralac," and the other filament-forming material may be a cellulose base material such as viscose. Both of these materials may be prepared in alkaline solution in a plastic form. The filament-forming material which is selected to constitute the dispersed phase of the composite will, as indicated above, be prepared with a sufficiently less fluid consistency so as to exist in the form of particles dispersed through the other, more fluid, material.

Various means for adjusting the fluidity of either of the filament-forming materials are available. The fluidity-reducing actions of coagulants and hardening agents appropriate to the various filament-forming materials are themselves well known, and can be employed in the preparation of the material that is to form the dispersed phase to reduce the fluidity of this material relative to the fluidity of the other material. Reduction of fluidity to such point as to prevent flow is of course to be avoided, since even the less fluid material should, as indicated above, still be plastic in order to flow through the orifices of the nozzle.

Difference in surface tension as between the two phases can best be enhanced by known means such as emulsification, such for instance as by incorporating small quantities of a water-immiscible oil in the material that is intended to form the dispersed phase, thereby to increase surface tension of particles of this material.

The length of time in which the two distinct phases are required to coexist in the material to be extruded of course depends upon the time elapsing between dispersion of the material of one phase in the material of the other phase and passage of the dispersed particles through the orifices of the extrusion nozzle. It is obvious that this time may be quite short.

The composite of the filament-forming materials is continuously fed to the plurality of adjacent orifices of an extrusion nozzle with the materials substantially uniformly disposed throughout the composite, and in passing through the individual orifices the particles of the less fluid filament-forming material at frequent intervals fill an individual orifice cross-section and temporarily exclude the other material, thereby alternating the materials that flow from a given orifice and staggering the staple filaments which emerge from the group of orifices of the nozzle. Thus in the accompanying drawing dispersed particles of, for instance, casein, indicated at C and shown in black, fill the cross sections of certain of the individual orifices of a spinneret 11 to the exclusion of the continuous phase filament-forming material, for instance viscose, indicated at V and shown as colorless, while at other individual orifices the continuous phase filament-forming material fills the cross sections of the orifices to the exclusion of the dispersed particles of casein. Thus separate staple lengths of casein SC (shown in black) and viscose SV (shown as colorless) are simultaneously produced, and are staggered and overlapped in the resulting sliver.

The extruded sliver emerging from the nozzle may then be subjected to a suitable hardening step, for instance by passing it into a bath 12 of sulphuric acid and formaldehyde adapted to harden both materials of the sliver.

Any tendency of the filament-forming materials to weld or stick together end to end during extrusion is obviated by the different surface tensions of the materials and/or by providing a gentle pull on the filaments as by flow of the fluid of the hardening bath along the filaments in their direction of departure from the nozzle.

The necessity for passage of inert or non-filament-forming material through the extrusion orifice as an interrupting agent is thus avoided, and a sliver consisting of a blend of filaments is expeditiously produced without the usual fiber-mixing processes.

I claim:

1. Method of forming a sliver of artificial fiber which comprises forming a composite comprising a filament-forming material in a continuous phase and another filament-forming material in a dispersed phase, both of said materials being in a flowable condition and being immiscible with each other so that each retains its separate identity, continuously feeding said composite to a plurality of adjacent orifices adapted to extrude the plurality of filaments which together constitute a sliver, said materials being so disposed substantially uniformly throughout the composite, as to present bodies of each material to the individual orifices at frequent intervals, such bodies of each filament-forming material filling the orifice cross section to the temporary exclusion of the other filament-forming material, thereby forming pieces of filament of staple length to produce a sliver from the several orifices comprising overlapped and longitudinally staggered pieces of both filament-forming materials.

2. Method of forming a sliver of artificial fiber in which a composite of flowable materials is fed through a plurality of adjacent orifices, and bodies of each material interrupt passage of the other material through the individual orifices, characterized in that both said materials comprise filament-forming materials, one said material being

in continuous phase and the other said material being in dispersed phase so that passage of each such body through an orifice forms such body into a staple length filament, and after passage through said orifices, both of said materials are subjected to hardening, to form a sliver.

3. Method of forming a sliver of artificial fiber in which a composite of flowable materials is fed through a plurality of adjacent orifices, and bodies of each material interrupt passage of the other material through the individual orifices, characterized in that both said materials comprise filament-forming materials, and are in alkaline condition, one said material being in continuous phase and the other said material being in dispersed phase, so that passage of each such body through an orifice forms such body into a staple length filament and after passage through said orifices, both of said materials are subjected to hardening in an acidic bath to form a sliver.

4. Method of forming a sliver of artificial fiber which comprises forming a composite comprising a filament-forming material and another filament-forming material, both of said materials being flowable and one of said materials being sufficiently less fluid than the other material so as to exist in the form of particles dispersed through the said other material, and continuously feeding said composite to a plurality of adjacent orifices adapted to extrude the plurality of filaments which together constitute a sliver, said particles of the less fluid filament-forming material at frequent intervals filling the individual orifice cross section to the temporary exclusion of the other material, thereby forming pieces of filament of staple length to produce a sliver from the several orifices comprising overlapped and longitudinally staggered pieces of both filament-forming materials.

5. Method of forming a sliver of artificial fiber which comprises forming a composite comprising a filament-forming material and another filament-forming material, both of said materials being in alkaline condition and being flowable and one of said materials being sufficiently less fluid than the other material so as to exist in the form of particles dispersed through the said other material, continuously feeding said composite to a plurality of adjacent orifices adapted to extrude the plurality of filaments which together constitute a sliver, said particles of the less fluid filament-forming material at frequent intervals filling the individual orifice cross section to the temporary exclusion of the other material, thereby forming pieces of filament of staple length to produce a sliver from the several orifices comprising overlapped and longitudinally staggered pieces of both filament-forming materials, and hardening the resulting filaments of the sliver by acid.

6. Method of forming a sliver of artificial fiber which comprises forming a composite comprising a protein filament-forming material and a cellulose base filament-forming material, both of said materials being in alkaline condition and being flowable and one of said materials being sufficiently less fluid than the other material so as to exist in the form of particles dispersed through the said other material, continuously feeding said composite to a plurality of adjacent orifices adapted to extrude the plurality of filaments which together constitute a sliver, said particles of the less fluid filament-forming material at frequent intervals filling the individual

orifice cross section to the temporary exclusion of the other material, thereby forming pieces of filament of staple length to produce a sliver from the several orifices comprising overlapped and longitudinally staggered pieces of both filament-forming materials, and hardening the resulting filaments of the sliver.

WILLIAM G. ABBOTT, JR.

REFERENCES CITED

10

The following references are of record in the file of this patent:

UNITED STATES PATENTS

| Number      | Name             | Date          |
|-------------|------------------|---------------|
| 2,331,945   | Pazsiczky et al. | Oct. 19, 1943 |
| 5 2,347,525 | Thinius          | Apr. 25, 1944 |

FOREIGN PATENTS

| Number  | Country       | Date          |
|---------|---------------|---------------|
| 483,731 | Great Britain | Apr. 21, 1938 |